

H. F. CLAYTON.  
PROCESS OF COATING WALLS AND OTHER SURFACES.  
APPLICATION FILED NOV. 5, 1915.  
**1,195,978.** Patented Aug. 29, 1916.



WITNESSES.

*N. R. Syndall.*  
*E. P. Hall.*

INVENTOR.

*H. F. Clayton*  
*By J. Edward Maybee.*  
ATTY.

# UNITED STATES PATENT OFFICE.

HARRY F. CLAYTON, OF TORONTO, ONTARIO, CANADA.

## PROCESS OF COATING WALLS AND OTHER SURFACES.

1,195,978.

Specification of Letters Patent. Patented Aug. 29, 1916.

Application filed November 5, 1915. Serial No. 59,799.

To all whom it may concern:

Be it known that I, HARRY F. CLAYTON, a subject of the King of Great Britain, residing in the city of Toronto, in the county of 5 York, Province of Ontario, Canada, have invented a certain new and useful Improved Process of Coating walls and other Surfaces, of which the following is a specification.

This invention relates particularly to the 10 treatment of walls or other stationary surfaces, which cannot be treated in furnaces, for the production thereon of a smooth glossy surface similar to that of enameled iron ware.

15 In carrying out my process I apply to the surface to be coated a finely ground fusible enamel or metallic powder mixed in water or other convenient liquid medium. For my purpose an easily fusible glass colored with 20 metallic oxids is well suited. One or more coats may be applied, if necessary, to give a sufficiently thick coating. The surface, when dry, is then subjected to the action of radiant heat at a very high temperature applied for 25 a sufficient length of time to fuse the coating without the effects of the heat extending below the surface. Such radiant heat at a sufficiently high temperature can be obtained by heating a plate of refractory material by 30 means of an oxy-acetylene blow pipe or electrically, and by moving this plate as slowly as may be necessary over the coated surface and at a distance determined by the temperature of the plate, the coating may be fused. 35 In the case of plaster, stucco, brick or tile walls and the like, the enamel coating may be applied direct to the surface with the certainty that it will adhere when fused. In the case of wood or other non-mineral surfaces, a mineral filling coat carried in a 40 liquid medium capable of readily penetrating the pores of the wood may be thoroughly worked into the surface before the enamel coat is applied. China clay mixed with oil 45 or glucose is suitable for this purpose. If a metallic coating be desired metallic powders suspended in any suitable medium, such for

example as the so called "banana oil," may be substituted for the enamel, and may be used either applied directly to the surfaces 50 or over a filling coat such as hereinbefore referred to.

A heater suited for my purpose is illustrated in the accompanying drawings in which—

Figure 1 is a longitudinal section of a suitable heating device; and Fig. 2 a front view of the same.

In the drawings like numerals of reference indicate corresponding parts in the different 60 figures.

1 represents a suitable casing lined with refractory material. The front of this casing is formed by a plate 2 of some suitable refractory material which is a good radiator 65 of heat. Graphite or carbon such as used for the manufacture of arc-light pencils is well suited for my purpose. This plate is located close to the front edge of the case and may be made adjustable to and from the 70 edge if necessary. Behind this plate is located an oxy-acetylene blow pipe 3 provided with a number of jets directed against the back of the plate. This will effectively heat the plate. Electrical or other means of 75 heating might, of course, be substituted. The back of the casing is provided with a handle 4 by means of which it may be moved as desired when in use.

What I claim as my invention is:

80 A process of coating surfaces *in situ* which consists in forming thereon a coating of a finely divided fusible mineral and thereafter fusing said coating by the action of radiant heat applied briefly and progressively to the 85 different parts of the surface from a portable source of relatively small area.

Signed at Toronto, this 22nd day of Oct. A. D. 1915, in the presence of the two undersigned witnesses.

HARRY F. CLAYTON.

Witnesses:

J. EDW. MAYBEE,  
E. P. HALL.